

# United States Patent [19]

Shiba et al.

[11] 3,920,458

[45] Nov. 18, 1975

[54] **PHOTOGRAPHIC SENSITIVE MATERIAL  
SUITABLE FOR THE SILVER-DYESTUFF  
BLEACHING METHOD**

[75] Inventors: Keisuke Shiba; Masanao Hinata,  
both of Minami-ashigara, Japan

[73] Assignee: Fuji Photo Film Co., Ltd., Japan

[22] Filed: Nov. 2, 1973

[21] Appl. No.: 412,521

**Related U.S. Application Data**

[63] Continuation of Ser. No. 184,585, Sept. 28, 1971,  
abandoned.

[30] **Foreign Application Priority Data**

Sept. 28, 1970 Japan ..... 45-84534

[52] U.S. Cl. .... 96/99; 96/124

[51] Int. Cl.<sup>2</sup> ..... G03C 1/10

[58] Field of Search ..... 96/99, 124

[56] **References Cited**

UNITED STATES PATENTS

|           |         |                  |              |
|-----------|---------|------------------|--------------|
| 3,157,507 | 11/1964 | Bruengger et al. | ..... 96/99  |
| 3,615,581 | 10/1971 | Kabitzke et al.  | ..... 96/99  |
| 3,617,293 | 11/1971 | Shiba et al.     | ..... 96/124 |
| 3,635,716 | 1/1972  | Bruengger et al. | ..... 96/99  |
| 3,682,640 | 8/1972  | Shiba et al.     | ..... 96/99  |
| 3,793,031 | 2/1974  | Shiba et al.     | ..... 96/99  |

Primary Examiner—J. Travis Brown  
Attorney, Agent, or Firm—Sughrue, Rothwell, Mion,  
Zinn & Macpeak

[57] **ABSTRACT**

A photographic sensitive material having at least one sensitive silver halide emulsion layer containing dyestuffs suitable for the silver-dyestuff bleaching

method, the improvement which comprises a combination of at least one of sensitizing dyestuffs of the following general Formula (I) and at least one of sensitizing dyestuffs of the following general Formula (II):



wherein Z represents a non-metallic atomic grouping required for the completion of a naphthothiazole or naphthoselenazole ring,  $Z_1$  represents a non-metallic atomic grouping required for the completion of a naphthothiazole, benzothiazole, naphthoselenazole or benzoselenazole ring, R represents a member selected from the first group consisting of a hydrogen atom, lower alkyl or aryl radical,  $R_1$  and  $R_2$  each represents an alkyl radical and at least one of said  $R_1$  and  $R_2$  is an alkyl radical containing a carboxyl or sulfo group, X represents an anion,  $n$  is 1 or 2, and  $n=1$  if an intermolecular salt is formed:



wherein  $Z_2$  and  $Z_3$ , which may be identical or different, each represents a non-metallic atomic grouping required for the completion of a benzothiazole or benzoselenazole ring,  $R_3$  represents a member selected from the second group consisting of a hydrogen atom, lower alkyl or aryl radical,  $R_4$  and  $R_5$  have the same meanings as  $R_1$  and  $R_2$  and at least one of said  $R_4$  and  $R_5$  is an alkyl radical containing a carboxyl or sulfo group, X represents an anion,  $m$  is 1 or 2, and  $m=1$  if an intermolecular salt is formed.

8 Claims, No Drawings

PHOTOGRAPHIC SENSITIVE MATERIAL  
SUITABLE FOR THE SILVER-DYESTUFF  
BLEACHING METHOD

This is a continuation, of application Ser. No. 184,585, filed Sept. 28, 1971, now abandoned.

FIELD OF THE INVENTION

This invention relates to an optical sensitization of photographic emulsions which contain dyestuffs suitable for the silver-dyestuff bleaching method and which is suitable for the method. In particular, it relates to the sensitization of red sensitive emulsions of the photographic sensitive material suitable for the silver-dyestuff bleaching method.

BACKGROUND OF THE INVENTION

One of the disadvantages in the silver-dyestuff bleaching method is that the sensitive rate of the dyed photographic layer is reduced to a considerable extent. The reason therefor is that the maximum sensitive wavelength is approximately identical to the maximum absorption wavelength of dyestuff. The sensitivity rate of the sensitive layer in the silver-dyestuff bleaching method is lower than that in other color photographic methods. Accordingly, a serious problem in the silver-dyestuff bleaching method is in the preparation of a layer having a sufficient sensitivity.

In the art of manufacturing a silver halide emulsion, it has been well known that the addition of sensitizing dyestuffs to the emulsion spreads the sensitive spectrum region of the emulsion resulting in an optically sensitized emulsion. The sensitizing dyestuffs used in the sensitive material for the silver-dyestuff bleaching method must satisfy some necessary requirements.

Except for the high sensitization, sensitizing dyestuffs should not cause residual coloration after the photographic sensitive material is treated. Further, sensitizing dyestuffs must be adsorbed firmly onto silver halide particles lest they must be substituted by dyestuffs suitable for the silver dyestuff bleaching method; otherwise the sensitizing effect is diminished highly by the presence of dyestuffs suitable for the silver dyestuff bleaching method.

A multi-layer material contains at least a blue sensitive emulsion layer, a green sensitive emulsion layer and a red sensitive emulsion layer. It is necessary that each color sensitization region of these three layers is separated well, above all that the red sensitive emulsion is as little green sensitive as possible. For this purpose, a red sensitive layer having a low green sensitivity and a high red sensitivity is required. The sensitizing dyestuff used in the red sensitive emulsion should not diffuse into other layers to provide the red sensitivity to them. The sensitizing dyestuff is apt to be desorbed from silver halide particles based on the presence of dyestuffs suitable for the silver-dyestuff bleaching method and diffused into other layers to provide the red sensitivity. A sensitizing method is required which does not show these characteristics.

An object of this invention is to provide a combination of sensitizing dyestuffs useful to the silver halide photographic emulsion used in the silver-dyestuff bleaching method and, in particular, to provide a photographic emulsion for the red sensitive layer, which has a high sensitivity and is substantially free from the residual coloration and does not provide the red sensi-

tivity to other layers. Other objects will be apparent to those skilled in the art as the description of this invention proceeds.

DESCRIPTION OF THE INVENTION

Objects of this invention are accomplished by using the combination of sensitizing dyestuffs represented by the following general Formula (I) and (II):



wherein Z represents a non-metallic atomic grouping required for the completion of a naphthothiazole or naphthoselenazole ring,  $Z_1$  represents a non-metallic atomic grouping required for the completion of naphthothiazole, benzothiazole, naphthoselenazole or benzoselenazole ring, R represents hydrogen atom, lower alkyl or aryl radical,  $R_1$  and  $R_2$  each represents alkyl radical such as, for example, methyl, ethyl, n-propyl,  $\beta$ -hydroxyethyl,  $\beta$ -acetoxyethyl and  $\gamma$ -acetoxypropyl radical, alkyl containing carboxyl group (for example, carboxymethyl,  $\beta$ -carboxyethyl and  $\gamma$ -carboxypropyl radical, 2-(2-carboxyethoxy)ethyl, alkyl containing sulfo group (for example,  $\beta$ -sulfoethyl,  $\gamma$ -sulfopropyl,  $\gamma$ -sulfobutyl,  $\delta$ -sulfobutyl, 2-hydroxy-1-sulfopropyl, 2-acetoxy-1-sulfopropyl, 2-(3-sulfopropoxy)ethyl, 3-methoxy-2-(3-sulfopropoxy)propyl, 2-(2-(3-sulfopropoxy)ethoxy)ethyl and 2-hydroxy-3-(3'-sulfopropoxy)propyl radical etc., and at least one of  $R_1$  and  $R_2$  is an alkyl radical containing carboxyl or sulfo group, X represents an anion,  $n$  is 1 or 2 and  $n=1$  if an intermolecular salt is formed.



wherein  $Z_2$  may be identical to or different from  $Z_3$  and each represents a non-metallic atomic grouping required for the completion of a benzothiazole or benzoselenazole ring,  $R_3$  represents a hydrogen atom, lower alkyl or aryl radical,  $R_4$  and  $R_5$  have the same meanings as  $R_1$  and  $R_2$ , and at least one of  $R_4$  and  $R_5$  represents an alkyl radical containing a carboxyl or sulfo group, X represents an anion,  $m$  is 1 or 2 and  $m=1$  if an intermolecular salt is formed.

Examples of naphthothiazole and naphthoselenazole rings which may be completed by Z and  $\alpha$ -naphthothiazole,  $\beta$ -naphthothiazole,  $\beta$ ,  $\beta$ -naphthothiazole,  $\alpha$ -naphthoselenazole,  $\beta$ -naphthoselenazole and  $\beta$ ,  $\beta$ -naphthoselenazole.

Examples of naphthothiazole, benzothiazole, naphthoselenazole and benzoselenazole rings which may be completed by  $Z_1$  are  $\alpha$ -naphthothiazole,  $\beta$ -naphthothiazole,  $\beta$ ,  $\beta$ -naphthothiazole, benzothiazole, 5-methylbenzothiazole, 5-chlorobenzothiazole, 5-methoxybenzothiazole, 5-bromobenzothiazole, 5,6-dimethylbenzothiazole, 5-cyanobenzothiazole, 5-phenylbenzothiazole, 5-hydroxy-6-methylbenzothiazole, 5-hydroxybenzothiazole, 5-ethoxy-6-methylbenzothiazole, 5-carboxybenzothiazole,  $\alpha$ -naphthoselenazole,  $\beta$ -naphthoselenazole,  $\beta$ ,  $\beta$ -naphthoselenazole, 5-methylbenzoselenazole, 5-chlorobenzoselenazole, 5-methoxybenzoselenazole, 5-phenylbenzoselenazole, 5,6-dimethylbenzoselenazole, 5-hydroxybenzoselenazole and the like.

Examples of R and R<sub>3</sub> as lower alkyl and aryl radicals are methyl, ethyl, n-propyl, phenyl, p-methoxyphenyl, o-carboxyphenyl and the like.

As examples of X, there may be mentioned chlorine, bromine, iodine, perchlorate, p-toluenesulfonic acid, 5 ethyl sulfuric acid ion etc.

The sensitizing dyestuffs to be used in this invention are known to those skilled in the art.

The combined use of sensitizing dyestuffs according to this invention provides a photographic emulsion having a low green sensitivity and a high red sensitivity in the presence of dyestuffs suitable for the silver dyestuff bleaching method. While, in the case of a red sensitive

emulsion in which a dyestuff of the Formula (I) or (II), alone is used, the dyestuff diffuses into another layer, for example, the green sensitive layer, to disadvantageously give the red sensitivity to the green sensitive layer. The combined use of dyestuffs according to this invention however, has the excellent characteristic of substantially not giving the red sensitivity to another layer.

Examples of sensitizing dyestuffs of the general Formula (I) used in this invention are shown as follows, but the sensitizing dyestuffs are not restricted only to these examples.

I-1



I-2



I-3



I-4



I-5



I-6



I-7



I-8



Examples of sensitizing dyestuffs of the general Formula (II) used in this invention are shown as follows, but the sensitizing dyestuffs are not restricted only to these examples.

II-1



II-2



II-3



II-4



II-5



II-6





The ratio of sensitizing dyestuff of the general Formula (I) to one of the Formula (II) used is not critical but an especially effective range is 9:1 – 1:9 by weight and may be varied according to the purpose for use.

The sensitizing dyestuffs of the general Formula (I) and (II) are introduced together with the dyestuff suitable for the silver-dyestuff bleaching method into the photographic layer used to the method. It is convenient to add the sensitizing dyestuffs to the emulsion, which has been washed with water and is not used for coating, especially before the addition of the dyestuff suitable for the method.

The process for the addition of said sensitizing dyestuffs to the photographic emulsion is well known in the field of manufacturing the emulsion. In general, it may be added as a solution in a solvent such as water, methanol, ethanol, methyl cellosolve, etc., to the photographic emulsion.

For the emulsion used in this invention, silver halide such as silver chloride, bromide, iodobromide, chlorobromide and chloroiodobromide may be used.

While a conventional gelatine-silver halide emulsion is used in this invention, resinous substances or cellulose derivatives which do not effect adversely to the sensitive material, may be used instead of gelatine.

The photographic emulsion used in this invention may contain conventional additives such as chemical sensitizer, anti-fogging agent, stabilizer, hardener, coating assistant, plasticizer, development accelerator and air anti-fogging agent.

The photographic emulsion may be coated in a common manner on a suitable supporter such as glass, film of cellulose derivate, a film of synthetic resin, a laminated paper, a synthetic paper and Baryta paper.

The dyestuffs which are used together with the sensitizing dyestuffs and which are suitable for the silver-dyestuff bleaching method are those which are used commonly in the method. In particular, those containing phenolic hydroxyl group or sulfonic acid group are preferred. Preferred dyestuffs are described in the specification U.S. Pat. No. 3,157,508.

was coated on a cellulose triacetate base. The treatment was carried out according to the following formulation. The results are shown in the Table 1.

|    |                                         |                   |
|----|-----------------------------------------|-------------------|
| 1. | Development for 5 min.                  |                   |
|    | p-methylaminophenol hydrochloride       | 1 g               |
|    | hydroquinone                            | 3 g               |
|    | anhydrous sodium sulfite                | 13 g              |
|    | potassium bromide                       | 1 g               |
|    | anhydrous sodium carbonate              | 26 g              |
|    | water                                   | enough to make up |
| 25 | Washing with water for 5 min.           | 1 l               |
| 30 | 3. Fixing for 5 min.                    |                   |
|    | crystalline sodium thiosulfate          | 200 g             |
|    | potassium metabisulfite                 | 20 g              |
|    | water                                   | 1 l               |
| 35 | 4. Washing with water for 5 min.        |                   |
| 40 | 5. Hardening for 5 min.                 |                   |
|    | 30% aq. solution of formaldehyde        | 100 ml            |
|    | anhydrous sodium carbonate              | 2 g               |
|    | water                                   | 1 l               |
| 45 | 6. Washing with water for 5 min.        |                   |
| 50 | 7. Bleaching the dyestuff for 10 min.   |                   |
|    | thiourea                                | 28 g              |
|    | potassium bromide                       | 18 g              |
|    | 2-amino-3-hydroxyphenazine              | 3 g               |
|    | conc. hydrochloric acid                 | 200 ml            |
|    | water                                   | 1 l               |
| 55 | 8. Washing with water for 5 min.        |                   |
| 60 | 9. Bleaching-fixing for 10 min.         |                   |
|    | tetrasodium ethylenediaminetetraacetate | 26 g              |
|    | anhydrous sodium carbonate              | 24 g              |
|    | ferric chloride                         | 15 g              |
|    | anhydrous sodium sulfite                | 13 g              |
|    | crystalline sodium thiosulfate          | 200 g             |
|    | water                                   | 1 l               |
| 65 | 10. Washing with water for 20 min.      |                   |

The structural formula of dyestuff used was as follows:



TABLE 1.

| Experimental No. | No. of Sensitizing Dyestuff-Amount of Dyestuff added (mg/silver halide g. mol) | Relative sensitivity (Red sensitivity) |
|------------------|--------------------------------------------------------------------------------|----------------------------------------|
| 1                | I-2(160) II-4(160)                                                             | 120                                    |
|                  | I-2(40) II-4(40)                                                               | 100                                    |
|                  | I-3(160)                                                                       | 165                                    |
|                  |                                                                                | 110                                    |

## EXAMPLE 1 – 6

Single sensitizing dyestuffs and combined ones were added respectively to a silver iodobromide emulsion (iodine content: 20 mol%) and stirred well for 20 minutes, and, after standing for a while, 19.0 g/silver halide / g mol of dyestuff of the following formula were added and stirred well, both common coating assistant and hardener were added and stirred well, and the whole

TABLE 1.-continued

| Experimental No. | Ex. No. | No. of Sensitizing Dyestuff-Amount of Dyestuff added (mg/silver halide g. mol) | Relative sensitivity (Red sensitivity) |
|------------------|---------|--------------------------------------------------------------------------------|----------------------------------------|
| 2                | 2       | I-3(40) II-5(160)                                                              | 100                                    |
|                  |         | I-6(160)                                                                       | 160                                    |
| 3                | 3       | I-6(20) II-1(160)                                                              | 100                                    |
|                  |         | I-6(160)                                                                       | 155                                    |
| 4                | 4       | I-6(20) II-7(160)                                                              | 100                                    |
|                  |         | I-8(160)                                                                       | 210                                    |
| 5                | 5       | I-8(20) II-8(160)                                                              | 26                                     |
|                  |         | II-6(160)                                                                      | 100                                    |
| 6                | 6       | II-6(40) II-5(20)                                                              | 160                                    |
|                  |         | II-5(160)                                                                      | 100                                    |
|                  |         | II-5(20)                                                                       | 170                                    |

What is claimed is:

1. In a photographic sensitive material having at least one red sensitive silver halide emulsion layer containing cyan azo dyestuffs suitable for the silver-dyestuff bleaching method, the improvement which comprises a combination of at least one of sensitizing dyestuffs of the following general Formula (I) and at least one of sensitizing dyestuffs of the following general Formula (II):



wherein Z represents a non-metallic atomic grouping required for the completion of a naphthothiazole or naphthoselenazole ring,  $Z_1$  represents a non-metallic atomic grouping required for the completion of a naphthothiazole, benzothiazole, naphthoselenazole or benzoselenazole ring, R represents a member selected from the first group consisting of a hydrogen atom, lower alkyl or aryl radical,  $R_1$  and  $R_2$  each represents an alkyl radical and at least one of said  $R_1$  and  $R_2$  is an alkyl radical containing a carboxyl or sulfo group, X represents an anion,  $n$  is 1 or 2, and  $n-1$  if an intermolecular salt is formed;



wherein  $Z_2$  and  $Z_3$ , which may be identical or different, each represents a non-metallic atomic grouping required for the completion of a benzothiazole or benzoselenazole ring,  $R_3$  represents a member selected from the second group consisting of a hydrogen atom, lower alkyl or aryl radical,  $R_4$  and  $R_5$  having the same meanings as  $R_1$  and  $R_2$  and at least one of said  $R_4$  and  $R_5$  is an alkyl radical containing a carboxyl or sulfo group, X represents an anion,  $m$  is 1 or 2, and  $m-1$  if an intermolecular salt is formed.

2. The photographic sensitive material according to claim 1 wherein the sensitizing dyestuff according to Formula (I) is selected from the group consisting of the following:



II-6



II-7



II-8



4. The photographic sensitive material according to claim 1 wherein said first and second group members are selected from the third group consisting of methyl, ethyl, n-propyl, phenyl, p-methoxyphenyl, and O - carboxyphenyl.

5. The photographic sensitive material according to claim 1 wherein said R<sub>1</sub>, R<sub>2</sub>, R<sub>3</sub> and R<sub>4</sub> radicals are se-

lected from the fourth group consisting of methyl, ethyl, n-propyl,  $\beta$ -hydroxyethyl,  $\beta$ -acetoxyethyl,  $\gamma$ -acetoxypropyl, carboxymethyl,  $\beta$ -carboxyethyl,  $\gamma$ -carboxypropyl, 2-(2-carboxyethoxy)ethyl,  $\beta$ -sulfoethyl,  $\gamma$ -sulfopropyl,  $\gamma$ -sulfobutyl,  $\delta$ -sulfobutyl, 2-hydroxy-1-sulfopropyl, 2-acetoxy-1-sulfopropyl, 2,(3-sulfo-propoxy)ethyl, 3-methoxy-2-(3-sulfopropoxy)propyl, 2-(2-(3-sulfopropoxy)ethoxy)ethyl and 2-hydroxy-3-(3'-sulfopropoxy)propyl.

6. The photographic sensitive material according to claim 1 wherein said X is selected from the fifth group consisting of chlorine, bromine, iodine, perchlorate, p-toluenesulfonic acid, and ethyl sulfuric acid.

7. The photographic sensitive material according to claim 1 wherein said Z is selected from the group consisting of  $\alpha$ -naphthothiazole,  $\beta$ -naphthothiazole,  $\beta$ , $\beta$ -naphthothiazole,  $\alpha$ -naphthoselenazole,  $\beta$ -naphthoselenazole, and  $\beta$ , $\beta$ -naphthoselenazole.

8. The photographic sensitive material according to claim 1 wherein said Z<sub>1</sub> is selected from the group consisting of  $\alpha$ -naphthothiazole,  $\beta$ -naphthothiazole,  $\beta$ , $\beta$ -naphthothiazole, benzothiazole, 5-methylbenzothiazole, 5-chlorobenzothiazole, 5-methoxybenzothiazole, 5-bromobenzothiazole, 5,6-dimethylbenzothiazole, 5-cyanobenzothiazole, 5-phenylbenzothiazole, 5-hydroxy-6-methylbenzothiazole, 5-hydroxybenzothiazole, 5-ethoxy-6-methylbenzothiazole, 5-carboxybenzothiazole,  $\alpha$ -naphthoselenazole,  $\beta$ -naphthoselenazole,  $\beta$ , $\beta$ -naphthoselenazole, 5-methylbenzoselenazole, 5-chlorobenzoselenazole, 5-methoxybenzoselenazole, 5-phenylbenzoselenazole, 5,6-dimethylbenzoselenazole, 5-hydroxybenzoselenazole.

\* \* \* \* \*

35

40

45

50

55

60

65